

## UNITED STATES PATENT OFFICE

2,584,041

PROCESS OF PREPARING OIL-SOLUBLE  
METAL SOAPS

Milton Nowak, Union, N. J., and Alfred Fischer,  
Bronx, N. Y., assignors to Nuodex Products Co.,  
Inc., Elizabeth, N. J., a corporation of New York

No Drawing. Application July 6, 1949,  
Serial No. 103,316

17 Claims. (Cl. 260—414)

1

This invention is directed to the preparation of oil-soluble metal soaps for use in the various arts. Heretofore such soaps have generally been produced, either through double decomposition processes employing the respective water-soluble salts of the metals and the water-soluble alkali soaps of the particular organic acids, or, by the reaction of the desired acids with thermally unstable compounds of the desired metals, such as carbonates, oxides and the like. Both of these conventional processes have recognized disadvantages. In the commercial practice of the double decomposition process, it is impossible to entirely free the end product oil-soluble metal soap from contamination by the by-product salts of such reactions, e. g., sodium sulphate. Another drawback to said process is the need of employing as an intermediate water-soluble salts of the specific metal. Such salts generally are more costly per metal content than the metal itself. Moreover, the equipment required for the practice of this process is complicated and relatively expensive. The thermal decomposition process can only be practiced with certain metals, but not all of them, and the economics are adverse because the cost of the metal content in the oxides and carbonates and the like is generally higher than of the metal itself.

Of the foregoing processes, the double decomposition reactions have commonly been referred to as the wet process and the thermal decomposition process is known as the dry process.

The object of the present invention is to eliminate the disadvantages of the aforesaid conventional processes and to permit the production of the desired end products through the use of more simple, highly efficient and economical process steps. We have been able to accomplish this result by a distinctively novel process which we term a hydrous two-phase acid-metal fusion, wherein the metal in comminuted form is reacted at elevated temperature with free organic acid in the presence of water.

An acid to be suitable within the teachings of this invention, must be capable of yielding water-insoluble, oil-soluble normal metal soaps. Examples of such acids are oleic acid, tall oil acids, naphthenic acids, 2-ethylhexoic acid, petroleum sulphonate acids, nonanoic acid, linseed oil fatty acids, soya bean oil fatty acids, phenyl stearic acids, and ether acids, such as butoxy butyric acid, etc. For commercial reasons, especially economic reasons and quality considerations, we prefer to use naphthenic acid, tall oil acid and 2-ethylhexoic acid, singly or in combination, but

we wish it to be understood that the scope of this invention is commensurate with the entire range of those substantially water-insoluble and substantially oil-soluble organic acids capable of forming oil-soluble heavy metal soaps.

While we are particularly concerned with the preparation of heavy metal soaps, we have also obtained satisfactory results with other metals, such as aluminum, strontium and the like. 10 Among the heavy metals which are of especial commercial importance, we have satisfactorily used: lead, cobalt, manganese, iron, copper, zinc, nickel, but we have also carried out preparation with many other members of the group of heavy metals.

Speaking generally, the process of this invention employs the metal preferably in powder form, in order that a large surface per weight is exposed to the reaction. The metal, together with 20 the selected organic acid and water, is maintained at elevated temperatures while thorough agitation is maintained. Under such conditions, there is a very complete and rapid conversion of the metal into the corresponding metal soap. 25 According to this invention, it is necessary to have water present throughout the entire reaction. This can be accomplished in various ways. For example, the process may be carried out under appropriate refluxing conditions. At the end of the reaction period, which in commercial practice may be a matter of a few hours, it is usually desired to remove the water. This can be accomplished by distilling it off or by mechanical means, e. g., centrifuging. In many instances, 30 we have found it desirable to employ water immiscible solvents for the end product. We have used mineral spirits, xylol and the like which are included within the reaction mass. The presence of such solvents often helps to facilitate the reaction and to reduce the viscosity of the end product, thus improving manipulation. In some cases, the reaction proceeded indifferently to the presence or absence of air, while in other cases the presence or absence of air affected the velocity 35 of the reaction.

40 It is sometimes desirable to employ certain modifying agents in minor amounts in order to impart certain characteristics to the end products. For example, the use of addition agents in amounts of as little as 1% may reduce the viscosity of the end product, which is desirable for certain applications. Moreover, certain of these agents serve to prevent oxidation and thus instability of the end product. The agents referred to may also be effective in improving the com-

3

patibility and stability of the end products in a broad range of other compositions into which they may be incorporated. By way of illustration, we may use the agents referred to in United States Patent No. 2,081,407 or those described in United States Reissue Patent No. 23,119. These agents may be added either before, during or after the reactions of this invention as they play no part in the reaction but are useful in modifying the properties of the end products.

Having thus generally described the present invention, we will now proceed with specific examples of practical performance.

#### EXAMPLE 1

##### *Cobalt naphthenate*

A solution of 530 grams of crude naphthenic acid (acid number 228) in 720 grams of mineral spirits is charged in a 2 liter, 3-neck, round bottom flask, equipped with agitator, reflux condenser, and an air inlet tube. The solution is agitated, and 100 grams of water added, together with 63 grams of finely powdered cobalt metal (95% cobalt content). The reaction mixture is heated to 195° F. and air is blown into the mixture at a rate of 25 liters per hour.

After 10 hours, the reaction is complete. The air inlet tube is closed, the reflux condenser removed, and the water present driven off by heating the reaction mixture to 220° F. The solution is then filtered to eliminate siliceous matter, analyzed for per cent oil-soluble cobalt, and diluted with mineral spirits to 6% cobalt. A conversion of 95% of the metal is obtained.

The end product is a dark blue-violet liquid consisting of a solution of cobalt naphthenate in mineral spirits and containing 6% cobalt. This material is useful as a catalyst in the drying of film-forming oxidizable material, as paints, varnishes, and the like.

#### EXAMPLE 1a

##### *Cobalt naphthenate*

A portion of the end product obtained in Example 1 is stripped of its volatile solvent by distillation in vacuum. The end product obtained is thus essentially free of any solvent and is a solid at room temperature.

#### EXAMPLE 1b

##### *Cobalt naphthenate with additives*

A cobalt naphthenate is prepared in exactly the same manner as described in Example 1, except that modifying agents are added to the end product reaction mass. Specifically 10 grams of triethanolamine lactate and 10 grams of amyl acid phosphate are added to the end products after the reaction is completed and prior to the driving off of the water. The addition of these modifying agents results in a cobalt naphthenate end product which is adapted for more universal use. The viscosity of the end product and resistance to oxidation are considerably improved over that of the straight cobalt naphthenate end product of Example 1.

#### EXAMPLE 2

##### *Cobalt tallate*

A solution of 325 grams of a commercial grade of tall oil (acid number 183, rosin acids content 37%) is dissolved in 310 grams of toluol, and charged in a 2 liter, 3-neck, round bottom flask, equipped with agitator, reflux condenser, and an air inlet tube. The solution is agitated, and

4

grams of water added with 31.5 grams of finely powdered cobalt metal (95% cobalt content). The reaction mixture is heated to 195° F. and air is blown into the mixture at a rate of 0.8 liter per minute.

After 12 hours, the reaction is complete. The water present is distilled off in vacuo, the solution filtered, analyzed, and diluted with toluol to 4% cobalt metal content. The yield is 720 grams (a conversion of 96% of the metal).

The end product is a dark violet colored liquid consisting of a solution of cobalt tallate in toluol, and may be employed as a drying catalyst in paints and varnishes.

#### EXAMPLE 3

##### *Cobalt 2-ethyl hexoate*

350 grams of 2-ethyl hexoic acid (acid number 380) are dissolved in 750 grams of mineral spirits, and placed in a 3 liter, 3-neck, round bottom flask, equipped with agitator, reflux condenser, and an air inlet tube. The solution is agitated vigorously, while 100 grams of water are added, together with 64.4 grams of powdered cobalt metal (92% cobalt content). The reaction mixture is heated to 175° F. and air passed into the mixture at the rate of 0.6 liter per minute. After 8 hours, the reaction is complete.

The water present is then distilled off, and the solution filtered to remove siliceous matter originally present in the cobalt metal. The solution is then analyzed, and diluted with mineral spirits to yield 728 grams of a solution of cobalt 2-ethyl hexoate containing 8% cobalt (97% conversion of the metal).

The product is a deep blue-violet liquid, useful as a drying catalyst in paints and varnishes.

40

#### EXAMPLE 4

##### *Manganese 2-ethyl hexoate*

380 grams of 2-ethyl hexoic acid (acid number 380) are mixed with 130 grams mineral spirits, and placed in a 3 liter, 2-neck, round bottom flask, equipped with agitator and reflux condenser. 60 grams of manganese metal flakes of approximately 4 mesh particle size are added to the solution, together with 60 grams water. The mixture is agitated rapidly, while heating to 212° F. The reaction is allowed to continue until all of the manganese metal has dissolved (approximately 10 hours).

The water present is then distilled off completely, together with some of the mineral spirits. The material is analyzed and diluted with mineral spirits to exactly 6% manganese metal content. A yield of 982 grams of manganese 2-ethyl hexoate solution of 6% metal content is obtained (98% yield).

This product is a dark amber liquid, and is useful as a catalyst in the drying of paints and varnishes.

65

#### EXAMPLE 5

##### *Manganese tallate*

685 grams of a commercial grade of tall oil (acid number 184, rosin acids content 37%), are mixed with 130 grams mineral spirits, and placed in a 3 liter, 2-neck, round bottom flask, equipped with agitator and reflux condenser. 60 grams of manganese metal powder (particle size: 98% through 300 mesh screen) are added to the solution, together with 60 grams of water. The mixture is agitated rapidly, while heating to 212°

## 5

F. The reaction is allowed to continue until all of the manganese metal has dissolved (approximately 2 hours).

The water present is then distilled off completely, together with some of the mineral spirits. The material is analyzed and diluted with mineral spirits to exactly 6% manganese metal content. A yield of 984 grams of manganese tallate solution of 6% metal content is obtained.

This product is a dark amber liquid, and is useful as a catalyst in the drying of paints and varnishes.

## EXAMPLE 6

*Manganese nonanoate*

361 grams of nonanoic acid (acid number 345) are mixed with 130 grams mineral spirits, and placed in a 3 liter, 2-neck, round bottom flask, equipped with agitation, and reflux condenser. 60 grams of manganese metal powder (particle size: 98% through 300 mesh screen) are added to the solution, together with 60 grams of water. The mixture is agitated rapidly, while heating to 212° F. The reaction is allowed to continue until all of the manganese metal has dissolved (approximately 2 hours).

The water present is then distilled off completely, together with some of the mineral spirits. There is then added 20 grams of nonanoic acid for the purpose of adjusting the viscosity and stability characteristics of the end product. The material is analyzed and diluted with mineral spirits to exactly 6% manganese metal content. A yield of 985 grams of manganese nonanoate solution of 6% metal content is obtained (98.5% yield).

This product is a dark amber liquid, and is useful as a catalyst in the drying of paints and varnishes.

## EXAMPLE 7

*Manganese naphthenate*

540 grams rectified naphthenic acid (acid number 230) are mixed with 130 grams mineral spirits, and placed in a 3 liter, 2-neck, round bottom flask, equipped with agitator and reflux condenser. 60 grams of manganese metal powder (particle size: 98% through 300 mesh screen) are added to the solution, together with 60 grams of water. The mixture is agitated rapidly, while heating to 212° F. The reaction is allowed to continue until all of the manganese metal has dissolved (approximately 2 hours).

The water present is then distilled off completely, together with some of the mineral spirits. The material is analyzed and diluted with mineral spirits to exactly 6% manganese metal content. A yield of 986 grams of manganese naphthenate solution of 6% metal content is obtained (98.6% yield).

This product is a dark amber liquid, and is useful as a catalyst in the drying of paints and varnishes.

## EXAMPLE 7a

*Manganese naphthenate with additive*

Preparation is carried out exactly in the same manner as set forth in Example 7, except that a modifying agent is added. Specifically 30 grams of isobutyl acid phosphate is added to the reaction mass prior to the stripping off of the water. The addition of the modifying agent results in a lowering of viscosity and improvement

## 6

of general performance over that of the end product of Example 7.

Instead of using the particular additive referred to, we have also used as an additive, amyl acid phosphate, triethyl citrate, tributyl citrate, etc. with satisfactory commercial results.

## EXAMPLE 8

*Copper oleate*

785 grams oleic acid (acid number 195) are dissolved in 600 grams mineral spirits, and placed in a 3-liter, round bottom flask, equipped with agitator, reflux condenser, and an air inlet tube. 100 grams water and 80 grams powdered copper metal (particle size: 98% through 325 mesh screen) are added to the acid solution and the reaction mixture then agitated rapidly. Temperature of the mixture is brought to 212° F. and air bubbled in at the rate of approximately 300 liters per hour.

After 14 hours, the reaction is substantially complete. The water is distilled from the mixture in vacuo, together with some of the mineral spirits. The reaction mixture is then filtered and analyzed for metal content. After analysis, it is diluted with mineral spirits to yield 900 grams of a solution of copper oleate containing 8% copper metal.

This product is a bright dark green liquid. It is useful as a pesticide in the preservation of cellulosic materials, as canvas, wood, etc.

## EXAMPLE 9

*Copper naphthenate*

665 grams crude naphthenic acid (acid number 228) are dissolved in 600 grams mineral spirits, and placed in a 3 liter, round bottom flask, equipped with agitator, reflux condenser, and an air inlet tube. 100 grams water and 80 grams powdered copper metal (particle size: 98% through 325 mesh screen) are added to the acid solution, and reaction mixture then agitated rapidly. Temperature of the mixture is brought to 212° F. and air bubbled in at the rate of approximately 300 liters per hour.

After 14 hours, the reaction is substantially complete. The water is distilled from the mixture in vacuo, together with some of the mineral spirits. The reaction mixture is then filtered and analyzed for metal content. After analysis, it is diluted with mineral spirits to yield 930 grams of a solution of copper naphthenate containing 8% copper metal.

The product is a bright dark green liquid. It is useful as a pesticide in the preservation of cellulosic materials, as canvas, woods, etc.

## EXAMPLE 10

*Copper tallate*

840 grams of a commercial grade of tall oil (acid number 183, rosin acids content 37%) are dissolved in 600 grams mineral spirits, and placed in a 3-liter, round bottom flask, equipped with agitator, reflux condenser, and an air inlet tube. 100 grams water and 80 grams powdered copper metal (particle size: 98% through 325 mesh screen) are added to the acid solution and reaction mixture then agitated rapidly. Temperature of the mixture is brought to 210° F. and air bubbled in at the rate of approximately 300 liters per hour.

After 14 hours, the reaction is substantially complete. The water is distilled from the mixture in vacuo, together with some of the mineral

7  
spirits. The reaction mixture is then filtered and analyzed for metal content. After analysis, it is diluted with mineral spirits to yield 1180 grams of a solution of copper tallate containing 6% copper metal.

This product is a bright dark green liquid. It is useful as a pesticide in the preservation of cellulosic materials, as canvas, wood, etc.

EXAMPLE 11

*Iron naphthenate*

172 grams crude naphthenic acid (acid number 230) are dissolved in 200 grams of xylol and charged in a 1 liter flask, equipped with agitator, reflux condenser, and air inlet tube. 40 grams water and 18 grams powdered iron (particle size: 98% through 200 mesh screen) are added to the solution, and the entire reaction mixture agitated rapidly. It is maintained at a temperature of 212° F. while air is blown into the mixture at a rate of approximately 60 liters per hour.

Reaction is found to be complete after 7 hours. The reaction mixture is placed in a separatory funnel, and the water drained off. The solvent layer is then dried completely by heating in vacuo, and the product is then filtered and analyzed for per cent iron. After analysis, the product is diluted with xylol to yield 415 grams of a solution of iron naphthenate in xylol containing 4% iron metal.

The end product is a very dark amber liquid useful as a drier in paints and varnishes.

EXAMPLE 12

*Manganese naphthenate*

575 grams of rectified naphthenic acid (acid number 230) are placed in a heavy duty mixer together with 60 grams of water. The reaction mixture is agitated and heated to 200° F. 60 grams of powdered manganese metal (particle size: 98% passing through 300 mesh screen) are added to the reaction mass and the agitation continued until all the manganese metal is reacted (approximately 5 hours). The water present is then distilled off completely by heating the mass to 220° F. The end product thus obtained represents solid manganese naphthenate of a metal content of approximately 10%.

EXAMPLE 13

*Iron tallate*

216 grams of a commercial grade of tall oil (acid number 183, rosin acids content 37%) are dissolved in 200 grams of mineral spirits and charged in a 1 liter flask, equipped with agitator, reflux condenser, and air inlet tube. 40 grams water and 18 grams powdered iron (particle size: 98% through 200 mesh screen) are added to the solution, and the entire reaction mixture agitated rapidly. It is maintained at a temperature of 212° F. while air is blown into the mixture at a rate of approximately 60 liters per hour.

Reaction is found to be complete after 7 hours. The reaction mixture is placed in a separatory funnel, and the water drained off. The solvent layer is then dried by heating in vacuo, and the product is then filtered and analyzed for per cent iron. After analysis, the product is diluted with mineral spirits to yield 425 grams of a solution of iron tallate in mineral spirits containing 4% iron metal.

8  
The end product is a very dark amber liquid useful as a drier in paints and varnishes.

EXAMPLE 14

*Iron 2-ethyl hexoate*

104 grams 2-ethyl hexoic acid (acid number 380) are dissolved in 250 grams xylol and placed in a 1 liter, 3-neck flask, equipped with reflux condenser, agitator, and air inlet tube. 35 grams of water and 18 grams powdered iron (particle size: 98% through 200 mesh screen) are added, and the reaction mixture agitated rapidly, while being maintained at a temperature of 212° F. Air is blown into the mixture at the rate of 50 liters per hour.

At the end of 6 hours the reaction is found to be substantially complete. The water present is distilled off, and the remaining solution filtered and analyzed for metal content. After analysis it is diluted to exactly 6% iron. Yield obtained is 288 grams.

The product is a very deep amber colored liquid.

EXAMPLE 15

*Zinc naphthenate*

665 grams rectified naphthenic acid (acid number 230) are dissolved in 600 grams mineral spirits, and placed in a 3 liter flask, equipped with agitator, reflux condenser, and air inlet tube. 100 grams of water, and 78 grams powdered zinc metal (particle size: 98% passing through a 300 mesh screen) are added, and the reaction mixture rapidly agitated. The temperature of the mixture is kept at 212° F., while air is blown in at the rate of 2 liters per minute. The reaction is completed after 6 hours.

The water is distilled off in vacuo, and the residue filtered and analyzed for per cent zinc. After analysis, the solution is diluted to 8% zinc content. A yield of 952 grams is obtained.

The product is a pale amber viscous liquid. It is useful as a wetting and grinding agent in the mixing of pigments, and as a pesticide and fungicide for the preservation of cellulosic materials.

EXAMPLE 16

*Zinc nonanoate*

445 grams of nonanoic acid (acid number 345) are dissolved in 600 grams mineral spirits, and placed in a 3 liter flask, equipped with agitator, reflux condenser, and air inlet tube. 100 grams of water, and 78 grams powdered zinc metal (particle size: 98% through 300 mesh screen) are added, and the reaction mixture rapidly agitated. The temperature of the mixture is kept at 212° F. while air is blown in at the rate of 2 liters per minute. The reaction is completed after 6 hours.

The water is distilled off in vacuo, and the residue filtered and analyzed for per cent zinc. After analysis, the solution is diluted to 8% zinc content. A conversion of 99% is obtained.

The product is a pale amber viscous liquid. It is useful as a wetting and grinding agent in the mixing of pigments, and as a pesticide and fungicide for the preservation of cellulosic materials.

EXAMPLE 17

*Zinc 2-ethyl hexoate*

403 grams 2-ethyl hexoic acid (acid number 380) are dissolved in 600 grams mineral spirits, and placed in a 3 liter flask, equipped with agitator, reflux condenser, and air inlet tube. 100 grams of water, and 78 grams powdered zinc

metal (particle size: 98% passing through 300 mesh screen) are added, and the reaction mixture rapidly agitated. The temperature of the mixture is kept at 212° F. while air is blown in at the rate of 2 liters per minute. The reaction is completed after 6 hours.

The water is distilled off in vacuo, and the residue filtered and analyzed for per cent zinc. After analysis, the solution is diluted to 10% zinc metal content. A conversion of 99% of the metal is obtained.

The product is a pale amber viscous liquid. It is useful as a wetting and grinding agent in the mixing of pigments, and as a pesticide and fungicide for the preservation of cellulosic materials.

#### EXAMPLE 18

##### *Lead naphthenate*

244 grams rectified naphthenic acid (acid number 230) are dissolved in 300 grams mineral spirits and solution placed in a 2 liter flask, equipped with reflux condenser, agitator and air inlet tube. 60 grams of water and 103.5 grams of finely powdered lead metal (particle size: 98% passing through 200 mesh screen) are then added to the reaction mixture and the entire mixture agitated rapidly and maintained at temperature of 212° F. Air is blown in at the rate of 90 liters per hour. After 12 hours, reaction is complete.

Water is distilled from the reaction mixture in vacuo, and the residue filtered and analyzed for lead content. After analysis, the solution is diluted with mineral spirits to exactly 16% lead metal content. A conversion of 97% of the metal is obtained.

This product consists essentially of a solution of neutral lead soap of naphthenic acid, and is an amber liquid. This material may be used as a drying catalyst in paints and varnishes.

#### EXAMPLE 19

##### *Basic lead naphthenate*

177 grams of rectified naphthenic acid (acid number 230) are dissolved in 150 grams mineral spirits, and placed in a 1 liter flask, equipped with reflux condenser, agitator, and air inlet tube. 60 grams of water, and 103.5° grams finely powdered lead metal (particle size: 98% passing through 200 mesh screen) are added to the reaction mixture, which is then rapidly agitated, and heated to a temperature of 212° F. Air is blown in at the rate of 3 liters per minute for a period of 15 hours, after which time the reaction is found to be substantially complete.

The water present is then distilled from the reaction mixture in vacuo. The remaining solution is then filtered and analyzed for lead content. After analysis, it is diluted with mineral spirits to yield 420 grams of a solution containing 24% lead metal.

This end product consists of a solution of basic lead naphthenate in mineral spirits. It is a clear light amber liquid, and is useful as a drying catalyst for paints and varnishes.

#### EXAMPLE 20

##### *Basic lead tallate*

122 grams of a refined grade of tall oil (acid number 183, rosin acids content 37%) are dissolved in 150 grams mineral spirits, and placed in a 1 liter flask, equipped with reflux condenser,

agitator, and air inlet tube. 60 grams of water, and 103.5 grams finely powdered lead metal (particle size: 98% passing through 200 mesh screen) are added to the reaction mixture, which is then rapidly agitated, and heated to a temperature of 212° F. Air is blown in at the rate of 3 liters per minute for a period of 15 hours, after which time the reaction is found to be substantially complete.

10 The water present is then distilled from the reaction mixture in vacuo. The remaining solution is then filtered and analyzed for lead content. After analysis, it is diluted with mineral spirits to yield 610 grams of a solution containing 16% lead metal:

This end product consists of a solution of basic lead tallate in mineral spirits. It is a clear light amber liquid, and is useful as a drying catalyst for paints and varnishes.

#### EXAMPLE 21

##### *Lead 2-ethyl hexoate*

148 grams 2-ethyl hexoic acid (acid number 380) are dissolved in 300 grams mineral spirits and solution placed in a 2 liter flask, equipped with reflux condenser, agitator, and air inlet tube. 60 grams of water and 103.5 grams of finely powdered lead metal (particle size: 98% passing through 200 mesh screen) are then added to the reaction mixture and the entire mass agitated rapidly and maintained at temperature of 212° F. Air is blown in at the rate of 90 liters per hour. After 12 hours, reaction is complete.

35 Water is distilled from the reaction mixture in vacuo, and the residue filtered and analyzed for lead content. After analysis, the solution is diluted with mineral spirits to exactly 24% lead metal content. A conversion of 97% of the metal is obtained.

This product consists essentially of a solution of a neutral lead soap of 2-ethyl hexoic acid, and is an amber liquid. This material may be used as a drying catalyst in paints and varnishes.

45

#### EXAMPLE 22

##### *Cobalt salt of a combination of tall oil and naphthenic acid*

50 250 grams naphthenic acid (acid number 228) and 310 grams of a commercial grade of tall oil (acid number 183, rosin acids content 37%) are dissolved in 720 grams mineral spirits and charged in a 2 liter, 3-neck, round bottom flask, equipped with agitator, reflux condenser, and an air inlet tube. The solution is agitated, and 100 grams of water added, together with 63 grams of finely powdered cobalt metal (95% cobalt content). The reaction mixture is heated to 195° F. and the air is blown into the mixture at a rate of 25 liters per hour.

60 After 10 hours the reaction is complete. The air inlet tube is closed, the reflux condenser removed, and the water present driven off by heating the reaction mixture to 220° F. The solution is then filtered to eliminate siliceous matter, analyzed for per cent soluble cobalt, and diluted with mineral spirits to 6% cobalt. A conversion of 96% of the metal is obtained.

65 70 The end product is a dark blue-violet liquid consisting of a solution of cobalt naphthenate-tallate in mineral spirits, and containing 6% cobalt. This material is useful as a catalyst in the drying of film-forming oxidizable material, as paints, varnishes, and the like.

## EXAMPLE 23

*Manganese salt of a combination of 2-ethyl hexoic acid and naphthenic acid*

168 grams 2-ethyl hexoic acid (acid number 380) and 278 grams rectified naphthenic acid (acid number 230) are mixed with 130 grams mineral spirits, and placed in a 3 liter, 2-neck, round bottom flask, equipped with agitator and reflux condenser. 60 grams of manganese metal flakes of approximately 4 mesh particle size are added to the solution, together with 60 grams water. The mixture is agitated rapidly, while heating to 212° F. The reaction is allowed to continue until all of the manganese metal has dissolved (approximately 10 hours).

The water present is then distilled off completely, together with some of the mineral spirits. The material is analyzed and diluted with mineral spirits to exactly 6% manganese metal content. A conversion of 99% of manganese metal is obtained.

This product is a dark amber liquid, and is useful as a catalyst in the drying of paints and varnishes.

## EXAMPLE 24

*Lead-cobalt naphthenate*

261 grams rectified naphthenic acid (acid number 230) are dissolved in 300 grams mineral spirits, and placed in a 2 liter flask, equipped with reflux condenser, agitator, and air inlet tube. To this solution are added 70 cc. water, 11.2 grams finely powdered cobalt metal (cobalt content 92%) (particle size: 98% passing through 325 mesh screen), and 103.5 grams of finely powdered lead metal (particle size: 98% passing through 200 mesh screen). The mixture is agitated rapidly, and maintained at a temperature of 212° F., while blowing in air at the rate of 4 liters per minute. After 15 hours, the reaction is substantially complete.

The water is distilled off in vacuo, and the reaction mixture then filtered and analyzed for percent soluble lead and cobalt. After analysis, it is diluted with mineral spirits to a lead content of 16% and a cobalt content of 1.6%. The conversion of each metal is approximately 93%.

The end product is a deep violet colored liquid, containing lead and cobalt in the ratio of 10:1; this ratio is one commonly employed where such metal combinations are used as drying catalysts in paints and varnishes.

## EXAMPLE 25

*Lead-cobalt salt of 2-ethyl hexoic acid and naphthenic acid*

177 grams rectified naphthenic acid (acid number 230) and 51 grams 2-ethyl hexoic acid (acid number 380) are dissolved in 300 grams mineral spirits, and placed in a 2 liter flask, equipped with reflux condenser, agitator, and air inlet tube. To this solution are added 70 cc. water, 11.2 grams finely powdered cobalt metal (cobalt content 92%) (particle size: 98% passing through 200 mesh screen). The mixture is agitated rapidly, and maintained at a temperature of 212° F., while blowing in air at the rate of 4 liters per minute. After 15 hours, the reaction is substantially complete.

The water is distilled off in vacuo, and the reaction mixture then filtered and analyzed for percent soluble lead and cobalt. After analysis, it is diluted with mineral spirits to a lead content of 16% and a cobalt content of 1.6%. The conversion of each metal is approximately 96%.

The end product is a deep violet colored liquid, containing lead and cobalt in the ratio of 10:1; this ratio is one commonly employed where such metal combinations are used as drying catalysts in paints and varnishes.

It will be apparent from the foregoing examples that a single acid and a single metal may be reacted in the manner stated or combinations of acids and/or metals may also be satisfactorily carried out. The invention is not limited to the illustrative examples given.

The end-products of this invention are suitable for many uses. They are highly satisfactory when used as catalysts for the drying of oxidizable film-forming materials, such as paints, varnishes and the like. They are also very effective as drying catalysts for printing inks. Another important field of application, particularly for the copper soaps, is that of pest control, including the conservation of wood and other cellulosic materials against the ravages of insects, fungi, etc. The end products may also be employed as coloring agents, e. g., as constituents of plastic compositions, to impart certain desirable colorization. Still another important utility is that of stabilizing certain plastics, such as vinyl plastics against decomposition. It is also quite practical to employ the heavy metal soaps themselves as film-forming agents. The end products of this invention may serve a great variety of purposes.

The foregoing examples refer to "naphthenic acid," "tall oil acid" and "tall oil." The raw materials so designated are the raw materials of the trade and all of such raw materials so sold on the open market will function properly in the examples given for the purpose of carrying out the present invention.

Having thus fully described the invention, what we claim as new and desire to secure by Letters Patent is:

1. The herein described hydrous two-phase metal-acid fusion process which comprises: commingling at least one comminuted polyvalent metal, at least one organic acid capable of forming oil-soluble heavy metal soaps, and a quantity of water to produce a reaction mass, and heating said mass to effect reaction thereof to a temperature above 100° F. under conditions to maintain the water in its liquid phase throughout the reaction while agitating the mass.
2. Process as claimed in claim 1, which includes the freeing of the oil-soluble metal soap end product from the water at the conclusion of the reaction.
3. The process of claim 1, wherein one metal is a heavy metal.
4. The process of claim 1, wherein one metal is a heavy metal and one acid is naphthenic acid.
5. The process of claim 1, wherein one metal is cobalt and one acid is naphthenic acid.
6. The process of claim 1, wherein one metal is cobalt and one acid is tall oil acid.
7. The process of claim 1, wherein one metal is cobalt and one acid is 2-ethylhexoic acid.
8. The process of claim 1, wherein one metal is manganese and one acid is naphthenic acid.
9. The process of claim 1, wherein one metal is manganese and one acid is tall oil acid.
10. The process of claim 1, wherein one metal is manganese and one acid is 2-ethylhexoic acid.
11. The process of claim 1, wherein one metal is iron and one acid is naphthenic acid.
12. The process of claim 1, wherein the metal is iron and one acid is tall oil acid.

13. The process of claim 1, wherein the metal is iron and one acid is 2-ethylhexoic acid.

14. The process of claim 1, wherein the metal is copper and one acid is naphthenic acid.

15. The process of claim 1, wherein the metal is copper and one acid is tall oil acid. 5

16. The process of claim 1, wherein the metal is copper and one acid is 2-ethylhexoic acid.

17. The herein described hydrous two-phase metal-acid fusion process which comprises: 10 commingling at least one comminuted polyvalent metal, at least one organic acid capable of forming oil-soluble heavy metal soaps, and a quantity of water to produce a reaction mass, and heating said mass in the presence of air to effect reaction thereof to a temperature above 100° F. under conditions to maintain the water in its liquid phase throughout the reaction while agitating the mass.

MILTON NOWAK. 20  
ALFRED FISCHER.

## REFERENCES CITED

The following references are of record in the file of this patent:

## UNITED STATES PATENTS

| Number    | Name         | Date          |
|-----------|--------------|---------------|
| 2,338,128 | Minich       | Jan. 4, 1944  |
| 2,397,767 | Taylor       | Apr. 2, 1946  |
| 2,409,678 | Hamblet      | Oct. 22, 1946 |
| 2,416,074 | Weber et al. | Feb. 18, 1947 |
| 2,423,619 | Roon         | July 8, 1947  |
| 2,445,935 | Bondi        | July 27, 1948 |
| 2,472,424 | Hoover       | June 7, 1949  |
| 2,527,789 | Bondi        | Oct. 31, 1950 |

## FOREIGN PATENTS

| Number  | Country       | Date          |
|---------|---------------|---------------|
| 589,242 | Great Britain | June 16, 1947 |